

## UNITED STATES PATENT OFFICE

2,515,803

## SULFONATED 1,1,1-TRICHLORO-2,2-BIS (p-CHLOROPHENYL) ETHANE

Ernest Segesemann, Woodridge, N. J., and  
Nicholas M. Molnar, New York, N. Y.No Drawing. Application May 17, 1945,  
Serial No. 594,364

1 Claim. (Cl. 260—505)

1

This invention relates, in general, to insecticidal agents and in particular to insecticidal agents which can be permanently impregnated into textile fabrics and other goods commonly used in wearing apparel or house furnishings.

We have discovered that by introducing an "auxochrome" group into the molecule of 1,1,1-trichloro-2,2-bis (p-chlorophenyl) ethane commonly known at DDT the compound can without losing its insecticidal properties be permanently attached onto organic fibres used for instance in textiles, as for example, textile fibres, wool, silk, cotton, rayon, or the like, or onto fur, feathers, or the like. In the case of animal fibres, such as wool, silk, feathers, fur, or the like, the compound will fix itself directly to the protein of the fibre while in the case of vegetable fibres, such as cotton rayon, or the like, permanent impregnation is accomplished with the help of mordants of the kind that are commonly used in the dyeing of vegetable fibres.

The fabrics or other goods thus treated are protected against damage from vermin such as moths, beetles and other insects and their larvae. The insecticidal effect is permanent and remains after repeated washing or drycleaning of the goods treated.

The term "auxochrome" group includes the groups or radicals known in dyestuff chemistry to possess the property of attaching the dyestuff firmly to the fibre. Such groups include for instance:



and the like.

A convenient method for imparting an auxochrome group into the molecule of DDT consists in introducing one or more sulfonic acid groups by treating DDT with sulfuric acid, chlorosulfonic acid or other sulfonating agents.

## Example #1

100 grams of DDT is suspended in 100 grams of chlorosulfonic acid and the mixture is stirred at a temperature of 40° to 50° C. until a sample of the reaction mass dissolves clearly in water. Usually a reaction time of 3 to 4 hours is required to effect complete sulfonation. The product of reaction is then poured into 500 ml. of water. Enough caustic soda or sodium carbonate is then added to neutralize the sulfonic acids and any free mineral acids. The product which consists of an aqueous solution of the sodium salt of DDT-sulfonic acids, sodium chloride and sodium sulfate may be used directly in its crude form for

the impregnation of textile fibres, fur, feathers, or the like, or it may be concentrated or evaporated to dryness or it may be freed from its inorganic impurities prior to its application to textile fibres.

2

## Example #2

60 ml. of the crude aqueous solution obtained in Example #1 were diluted to 100 ml. with water. 10 To this solution was then added 5 grams of sodium sulfate and 3 ml. of glacial acetic acid. The solution was then heated to 40° C. and a piece of knitted wool weighing 15 grams was introduced. The temperature was then gradually raised at 15 such a rate that it came to a boil after 20 minutes. The bath was then kept boiling for one hour. 1.5 ml. of sulfuric acid was then added and boiling was continued for an additional 30 minutes. The wool was then rinsed thoroughly with fresh 20 water and dried.

The treated wool was then exposed to the larvae of moths and of the black carpet beetle for three weeks without being attacked by the vermin; while untreated pieces of wool used as controls 25 were freely fed upon by the larvae. The exposure tests were repeated after the piece of treated wool had been washed six times. Again the wool remained unattacked by the vermin.

The piece of treated wool was then put through 30 a drycleaning process using Stoddard solvent and a commercial dry-cleaning soap. Tests on the larvae of moths and black carpet beetle were again negative indicating that the fabric had retained its insecticidal or insect repellent quality.

35

## Example #3

20 grams of DDT was suspended in 25 grams of Oleum containing 20% free SO<sub>3</sub> and stirred at 40 80° C. for 5 hours. The reaction mixture was poured into 300 ml. of water and neutralized with 45 caustic soda. The solution was then filtered off from a small quantity of unreacted material and the filtrate was then evaporated to dryness. The solid mass which consisted of the sodium salts of DDT sulfonic acids, and sodium sulfate was ground to a powder and extracted with 3 portions each of 50 ml. of methanol. The filtered extract was then evaporated to dryness. The product consisting of the pure sodium salts of DDT sulfonic acids is a light yellow solid which can be 50 ground to a powder.

Fabrics impregnated in accordance with the procedure described in Example #2 were completely protected against damage by the larvae 55 of moths or those of the black carpet beetle.

## Example #4

20 grams of DDT were dissolved in 30 ml. of ethylenedichloride and 20 grams of chlorosulfonic acid was then added. The mixture was kept at 50° C. for 12 hours and was then cooled at 0° C. for 8 hours. The free sulfonic acids of DDT which crystallized out were then filtered off and washed with a small quantity of cold ethylenedichloride.

## Example #5

20 grams of DDT were dissolved in 30 ml. of ethylenedichloride and 20 grams of chlorosulfonic acid was then added. The mixture was allowed to stand at 50° C. over night. The mass was then poured into 200 ml. of water and well agitated. The solvent layer was allowed to settle to the bottom and was then drawn off and discarded. The aqueous solution was then neutralized with caustic soda and was then evaporated to dryness. The dry cake was ground to a powder and was then extracted with 4 portions of 50 ml. each of absolute ethanol. The combined ethanol extracts were then concentrated to dryness by distilling off the alcohol. The light yellow product was then ground to a powder.

A piece of white cotton fabric weighing 10 grams was soaked in 100 ml. of a 1% aqueous solution of sulfonated castor oil. The fabric was then squeezed and immersed in 100 ml. of an aqueous bath containing 1 gram of aluminum sulfate, 2 grams of a 30° Be. solution of sodium bisulfite, 0.5 gram of calcium acetate, 1 gram of sodium chloride and 1 gram of sodium salts of

DDT sulfonic acids as obtained in the above procedure. The bath was slow-brought to the boiling point and kept boiling for 1 hour. The fabric was then well rinsed with fresh water and dried.

The piece of treated cotton was then placed into a test jar containing six cat fleas. All the fleas were dead after three hours.

Having described our invention, what we claim and desire to secure by Letters Patent, is as follows:

A new compound, 1,1,1-trichloro-2,2-bis(p-chlorophenyl)ethane being at least once substituted by a sulfonic acid group.

ERNEST SEGESSEMAN. NICHOLAS M. MOLNAR.

## REFERENCES CITED

The following references are of record in the file of this patent:

## UNITED STATES PATENTS

| Number     | Name           | Date          |
|------------|----------------|---------------|
| Re. 22,700 | Muller         | Dec. 4, 1945  |
| 1,707,181  | Weiler         | Mar. 26, 1929 |
| 1,887,958  | Schwen et al.  | Nov. 15, 1932 |
| 2,053,610  | Hermann et al. | Sept. 8, 1936 |
| 2,329,074  | Muller         | Sept. 7, 1943 |

## OTHER REFERENCES

Aickin, "Adsorption of Sodium Alkyl Sulfates by Wool and Other Fibers," J. Soc. Dyers & Col. 1944, No. 3, pp. 60-65.

Karrer, "Organic Chemistry," 2nd Engl. Ed., 1946, Elsevier Publ. Co., N. Y. (based on 8th Germ. ed. Leipzig, 1942), pp. 468-469.